

(No Model.)

PEDRO DEL VALLE.

PROCESS OF SEPARATING METALS BY AMALGAMATION.

No. 416,403.

Patented Dec. 3, 1889.



WITNESSES:

Fred G. Dieterich  
Jos. A. Ryan

INVENTOR

Pedro del Valle

BY Alfredo L.

ATTORNEY

# UNITED STATES PATENT OFFICE.

PEDRO DEL VALLE, OF MEXICO, MEXICO.

## PROCESS OF SEPARATING METALS BY AMALGAMATION.

SPECIFICATION forming part of Letters Patent No. 416,403, dated December 3, 1889.

Application filed June 22, 1888. Serial No. 277,936. (No model.)

*To all whom it may concern:*

Be it known that I, PEDRO DEL VALLE, a citizen of the Mexican Republic, residing in the city of Mexico, the capital of said Republic, have invented a new and useful Improvement 5 in the Process of Separating Metals by Amalgamation, (which improvement is fully set forth in the following specification;) and I do hereby declare that the following is a clear and exact description of the invention, which will enable others skilled in the art to which it appertains to make and use the same, reference being had to the accompanying drawing, forming part of this specification, which shows a vertical section of the apparatus for carrying out my process.

My invention consists in the improved process hereinafter described and claimed.

In the drawing, X is a suitable inclosing- 20 tank having vertical partitions Y and Z, and which tank is to be provided with a body of mercury which rises to the level of the line a.

Outside of partition Y is disposed a pump consisting of a cylinder A, with downwardly- 25 opening valve B at the bottom, and a piston with downwardly-opening valves B' B<sup>2</sup>. In the place of this pump there may be used other kinds of machines for injecting into the lower part of the mercury the pulverized or 30 calcined ore, either alone or mixed with convenient substances for amalgamation.

C are horizontal plates fixed in the partitions Y and Z, and having openings b alternately at opposite ends.

35 D E is a circulating mercury-pump, opening both above and below the plates C.

F is the outlet for the discharge of amalgamated metals.

S are screens or wire sieves placed between 40 the horizontal plates C.

The arrows in full lines indicate the endless course of the mercury stream raised and circulated by the pump D E.

The dotted arrows indicate the course of the 45 ore stream.

The crossed arrows indicate the course of the metals and amalgams of greater specific

gravity than mercury, which, descending to the bottom, escape at F.

The operation is as follows: The apparatus 50 will be put in a pan with the required quantity of pure or amalgamated mercury, or mercury mixed with any other convenient substance. Through the tube or pump A, with the valve B, the pulverized ore is injected 55 into the lower part of the mercury beneath the plates C. The particles of metals and amalgams in the ore injected, of greater specific gravity than mercury, will go down to the bottom of the mercury and can be easily 60 collected. They are marked in the drawing by the crossed arrows, thus . The remaining particles of the ore injected, which are of less specific gravity than mercury, will ascend to the surface of the mercury, passing 65 on the way between the horizontal plates C and through the openings b. This will form the ascending ore stream, marked by dotted arrows, which, after reaching the upper surface of the mercury, will flow out of the apparatus at H. Between the plates C several 70 wire screens S will be placed, in order that the ascending pulverized ore stream when passing through them may be divided and subdivided within the mercury and its particles put 75 in intimate contact with the mercury and mixed with it, in order to obtain complete amalgamation. By the pump D E the mercury from the lower part of the tank will be raised to the upper part of the charge of mercury, in 80 order that the mercury stream, marked by the full arrows, when descending by the way between the plates C and through the screens, will be in contact and mixed with the particles of the pulverized ore stream ascending 85 by the same way. The pulverized ore, after having been passed through the apparatus, can be passed again several times and mixed, and, if desired, may be calcined and mixed with some appropriate substances until satisfactorily reduced.

I am aware of the patent to H. J. Smith, dated July 9, 1867, in which the ore and the mercury are circulated horizontally in oppo-

site directions through a cylinder provided with revolving perforated disks, and I do not claim such process or construction.

Having thus described my invention, what I claim as new is—

The process herein described of separating and amalgamating metals by establishing a downward circulation of mercury through an ascending stream of pulverized ore and elimi-

nating or drawing off the heavier metals to and amalgams which gravitate out of the circulation, substantially as shown and described.

Mexico, May 14, 1888.

PEDRO DEL VALLE.

Witnesses:

M. VICARIO DE LA RIVERA,  
ANDRES FALLE.